

No. 774,304.

PATENTED NOV. 8, 1904.

M. P. BOSS.  
METALLURGICAL PROCESS.  
APPLICATION FILED AUG. 6, 1903.



WITNESSES:

J. E. Pearson  
Frank O'Connor

INVENTOR

M. P. Boss  
BY  
Grover & Brinckmann  
ATTORNEY

## UNITED STATES PATENT OFFICE.

MARTIN PRIOR BOSS, OF SAN FRANCISCO, CALIFORNIA.

## METALLURGICAL PROCESS.

SPECIFICATION forming part of Letters Patent No. 774,304, dated November 8, 1904.

Application filed August 6, 1903. Serial No. 168,464. (No specimens.)

*To all whom it may concern:*

Be it known that I, MARTIN PRIOR Boss, a citizen of the United States, residing at San Francisco, county of San Francisco, State of California, have invented certain new and useful Improvements in Metallurgical Processes, of which the following is a specification.

This invention relates to a method of converting iron ore into steel continuously with-  
in a single furnace structure and depends upon the observed fact that in a furnace heated by a hydrocarbon fuel a hydrocarbon vapor may exist which is not consumed, but will combine with a heated metal when the two are brought in contact.

The object of my invention is to reduce the cost of obtaining steel from an iron ore.

The accompanying drawings will serve to illustrate such a furnace as may be employed to carry my invention into effect.

Figure 1 is a plan view. Fig. 2 is a section on the line 2 2 of Fig. 1. Fig. 3 is a section on the line 3 3 of Fig. 2. Fig. 4 is a section on the line 4 4 of Fig. 2.

The furnace which is shown consists of an inclined chamber A and a horizontal chamber B. The hearth of the chamber A is preferably formed of refractory bricks C, located one upon the other and in such manner that the successive bricks will form a series of steps. The purpose of this construction is to form a series of surfaces which normally tend to check sliding of the ore-body from the point of entrance to the point of delivery of the molten metal upon the hearth of the chamber B. This construction, however, is not essential and may be done away with. The hearth of the chamber B is also shown as inclined from the rear end toward the discharge-spout D. Preferably this hearth E is formed of sand or other refractory material.

Located at the top of the chamber A is a hopper F, through which the ore to be treated is introduced. Located under the hopper and so situated as to direct a flame of gas and air in a downward direction along the chamber A are the gas and air burners G. Any suitable gas and air burners may be employed.

I may use a burner adapted to operate with a hydrocarbon oil or a producer-gas.

Located under the burners G are a series of pushing-screws H, which project at their forward ends into a chamber A. Passing through these screws are oil-pipes I. The object of the screws is to push the ore from without inward and downward along the inclined hearth C, at the same time feed into the ore-body through the oil-pipes I a certain amount of oil, which I find to be an advantage and to aid in the decomposition or reduction of the ore.

Connected to the forward end of the chamber B is a flue J, which communicates with the stack K. Located in the stack K is a vertical-tube boiler L. The boiler may be dispensed with.

M indicates a slag-door in the chamber B; N, a door through which access may be obtained to the top of the molten metal on the hearth E of the chamber B; O, a door in the chamber A, through which air may be admitted.

The general method of operation is as follows: The ore is introduced through the hopper F and drops upon the hearth C of the chamber A. Here it is subjected to the reducing action of the hydrocarbon fuel introduced through the burners G and the pipes I. As the ore is reduced it melts and flows down the inclined hearth C and onto the hearth E of the chamber B. During the passage of the ore toward the chamber B it is brought into contact with a hydrocarbon vapor from the fuel introduced through the burners G and pipes I. This vapor combines with the iron ore under treatment with the result that steel having the required proportion of carbon is directly produced.

Having thus described my invention, I claim—

1. The herein-described method of producing steel direct from iron ore, which consists in subjecting the ore to the reducing action of a hydrocarbon-flame, and at the same time to the combining action of a hydrocarbon vapor.
2. The herein-described method of producing steel direct from iron ore, which consists

in reducing the ore to a molten metallic state by the action of a hydrocarbon-flame, and simultaneously subjecting the molten metal to the combining action of a hydrocarbon vapor.

5 3. The herein-described method of converting an iron ore into steel, which consists in discharging the iron ore upon an inclined and heated hearth, and discharging over said ore along its direction of movement a body of hydrocarbon gas and air in excess of that required for combustion.

15 4. The herein-described method of converting an iron ore into steel, which consists in discharging the iron ore upon an inclined and heated hearth, and discharging over said ore along its direction of movement a stream of ignited hydrocarbon gas and air, and wherein in the hydrocarbon gas is in excess of the amount required for combustion.

20 5. The herein-described method of reducing an ore-body and introducing carbon into the metal extracted therefrom in sufficient amount to convert it into steel, which consists in subjecting the ore-body to the action of a hydro-

carbon-flame, and the metal extracted therefrom to the action of a highly-heated free hydrocarbon vapor.

6. The herein-described method of reducing an ore-body, which consists in discharging it upon an inclined and heated hearth, introducing into it a hydrocarbon-body in sufficient amount to convert it into steel, and subjecting it during its passage over said hearth to the action of flame.

7. The herein-described method of reducing an ore-body, which consists in discharging it upon an inclined and heated hearth, introducing into it a hydrocarbon-body in sufficient amount to convert it into steel, and subjecting it during its passage over said hearth to the action of flame and a hydrocarbon vapor.

In testimony whereof I affix my signature in the presence of two witnesses.

MARTIN PRIOR BOSS.

Witnesses:

HENRY C. DROGER,  
JAMES L. KING.